

Oct. 26, 1937.

C. C. TOWNE

2,097,245

LUBRICATING OIL

Filed March 7, 1934



Charles C. Towne  
INVENTOR  
BY *R. J. Neelbom*  
HIS ATTORNEY

## UNITED STATES PATENT OFFICE

2,097,245

## LUBRICATING OIL

Charles C. Towne, Poughkeepsie, N. Y., assignor  
to The Texas Company, New York, N. Y., a  
corporation of Delaware

Application March 7, 1934, Serial No. 714,360

14 Claims. (Cl. 196—10)

This invention relates to the manufacture of petroleum lubricating oils, and particularly oils of this character possessing a green fluorescence and other desirable properties.

5 One of the objects of this invention is to provide a petroleum lubricating oil possessing a green fluorescence from a distillate oil which is normally deficient in that property, by utilization of cheap or normally waste materials available at oil 10 refineries, such as fixed refinery gases or oil gas from cracking stills.

Another object of the invention is to provide a method of preparing a green bloom material from normally gaseous hydrocarbons of this character.

15 Another object of the invention is to provide a pour point depressant for a mineral oil from gaseous hydrocarbons of this character, and a lubricating oil having a low pour point from a partially dewaxed oil by utilization of such pour point 20 depressant.

25 Still another object of the invention is to provide a method of dewaxing a wax bearing oil by the employment of a wax crystal modifying material obtained from gaseous hydrocarbons of this character.

It is well known that certain distillate lubricating oils, which are of excellent quality as lubricants, are nevertheless deficient in the property of bloom. Certain Pennsylvania lubricating 30 oils are reddish-brown by transmitted light and green by reflected light, thereby possessing what is termed a green bloom or fluorescence. In certain instances, it has been considered desirable to impart to lubricating oil distillates which are 35 deficient in this property of bloom, a green fluorescence similar to that which is characteristic of Pennsylvania base oils. It has heretofore been suggested that a green bloom imparting material can be prepared from the residuum of distillation, 40 either cracking or non-cracking, of a petroleum oil. However, this has necessitated the employment, as starting materials, of mineral oils which could otherwise be used for the preparation of more valuable products. Furthermore, this has 45 necessitated special distillation equipment and processing, in order to produce a bloom imparting material of acceptable character.

I have discovered that a very satisfactory green bloom imparting material may be prepared from 50 hydrocarbon gases, such as oil gas from cracking stills, or other waste gases from oil refineries. Other hydrocarbon gases of a similar nature, such as natural gases, fixed gases from the stabilization of natural gasoline, storage relief gases, as 55 well as individual constituents thereof including

propane, butane, etc., and mixtures thereof, may be employed for this purpose.

According to the present invention, the hydrocarbon gases are subjected to high temperature 5 pyrolysis in a cracking still. This may be accomplished in connection with a plant for the manufacture of benzol and its homologues from hydrocarbon gases by pyrolysis thereof, in accordance with my Patent No. 1,943,246 dated January 9, 1934. "High temperature" pyrolysis has the usual

10 significance of this term in the art,—namely, a pyrolysis in which the gases are passed through a heating coil or zone at a temperature in excess of 1150° F., and generally at temperatures varying between 1150°—2000° F. Known types of cat-

15 catalysts may be employed, either as porous catalysts within the heating tubes, or as materials constituting the heating tubes. The gases may be maintained at substantially atmospheric pressure, or they may be passed through the heating 20 coil under superatmospheric pressures varying up to 500 lbs. per sq. in. or higher. The pyrolyzed gases are then passed to a cooling zone, such as a water cooled condenser, where the temperature 25 is controlled to separate primarily high boiling constituents, mainly above the boiling points of benzol and homologous hydrocarbons of the benzene series. In this manner, there is condensed a liquid fraction comprising a heavy black oil.

Depending upon the temperature of condensation, this material will usually comprise a small proportion of benzol and naphthalene in admixture with a tarry residue. The latter is found to be highly concentrated in green bloom 30 imparting material. The condensate oil may be 35 mixed directly with a mineral lubricating oil to impart a green fluorescence thereto; or a concentrated extract of bloom imparting material may be obtained from the condensate oil by suitable methods, such as distillation or solvent extraction, and the concentrated extract then added 40 to a mineral lubricating oil.

45 Referring to the drawing, in which the single figure is a diagrammatic view of apparatus for carrying out the method of this invention, 10 indicates a cracking furnace containing a coil 11 through which the hydrocarbon gas is passed and heated to a high temperature such as ordinarily used in gas pyrolysis operations. The products of pyrolysis are discharged into a water 50 cooled condenser 12, to which cooling water is supplied by line 13 and discharged by line 14.

The products pass upwardly through tubes 15 of the condenser, uncondensed gases escaping by pipe 16 leading to a fractionating tower 17 where 55

80

85

90

95

100

105

110

various lower boiling constituents, including benzol, may be separated. The gas outlet temperature of the condenser 12 is preferably controlled to about 400° F. or above, so that mainly high boiling constituents are condensed therein. These constituents form a black oil which runs down the tubes 15, accumulating in the lower portion of the condenser, and discharging by the line 20. Although normally solid compounds are present in this oil, the liquid constituents maintain them in solution, and clogging of the condenser does not occur.

This condensed oil may be added directly to a mineral lubricating oil to impart a green bloom 15 to the latter. Or, if desired, the condensed oil may be treated or purified prior to use, such as by simple filtration, or by heating in contact with an adsorbent material followed by filtration, or by acid treatment or other conventional treatments 20 employed in the refining of petroleum oils. This is indicated in the drawing, in which the pipe 20 discharges into a refining tank 21 to which suitable chemical may be introduced by pipe 22. If desired, the oil may be treated to 25 prepare a concentrate therefrom; as it is found that the bloom imparting materials in the oil consist mainly of high boiling constituents which remain in the tarry residue resulting from reducing the oil by distillation, or are dissolved 30 from the oil or residue by solvent extraction. However, it is not necessary that any of these refining or concentrating treatments be employed, as the condensate recovered from condenser 12 may be satisfactorily marketed as a bloom im- 35 parting material.

The condensate, whether treated or not in the refining tank 21, is passed by line 24 to either valve controlled line 25 leading to receiver 26, or valve controlled line 27 leading to receiver 28. 40 From the receivers 26 and 28, the bloom oil or concentrate is passed by lines 29 and 30 respectively to a blending tank 32, to which the lubricating oil to be treated is admitted by line 33. Only a small proportion of the bloom oil or 45 concentrate need be added to a mineral lubricating oil to impart a satisfactory green fluorescence thereto. Thus, less than 2% by weight of the condensate as obtained from condenser 12, or even a smaller proportion of extract prepared 50 therefrom, is ordinarily employed in blending with a distillate lubricating oil. The blended oil is then passed by line 35 to storage tank 36, from which it is withdrawn for use or further treatment by line 37.

55 As a specific example of the present invention, an oil gas obtained from vapor phase cracking stills, is passed through a silica tube 20 mm. in diameter by 48 in. in length at the rate of 0.6 cu. ft. per hour, the tube being maintained at a 60 temperature of 1450°-1500° F. Issuing vapors are cooled in a water cooled condenser having a vapor outlet temperature of approximately 450° F. A black condensate oil is thereby obtained in the amount of approximately 10 cc. per 4 to 5 cu. ft. 65 of gas treated. 0.25 cc. of this oil dissolved in 100 cc. of a pale Mid-Continent distillate lubricating oil (Saybolt viscosity 300 at 100° F.) so altered the appearance and bloom of the distillate oil that it resembled a natural paraffin base cylinder stock.

70 It has further been found that the shade of the bloom imparted to pale lubricating oils by the product of this invention varies with the temperature at which the latter is prepared. For 75 example, where an oil gas from a vapor phase

cracking still is pyrolyzed at a temperature of approximately 1450°-1500° F., and a condensate oil recovered therefrom in the manner described above, the green bloom imparted to a mineral distillate oil is found to possess a slight bluish tinge. On the other hand, where the same oil gas is passed through the same cracking still at a temperature of approximately 1600°-1700° F., the condensate oil recovered therefrom, when added to the same pale lubricating oil, imparts a 10 green bloom which has a somewhat yellower tinge than that of a usual Pennsylvania oil. By blending in suitable proportions the condensate oils prepared at different temperatures, and adding the blend to a distillate oil, a resulting bloom 15 is obtained which approaches very closely the green bloom of a customary Pennsylvania oil, while at the same time the reddish-brown color by transmitted light is substantially the same. The heat treatments at different temperatures 20 may be accomplished in separate cracking stills. Or, as shown, a single cracking still may be employed; and a certain proportion of oil gas passed through the furnace 10 at one temperature, the condensate oil 25 being collected in one of the receivers 26 or 28, and then another portion of oil gas passed through the cracking furnace 10 at a different temperature, the condensate oil therefrom being collected in the other receiver. The resulting bloom oils may then be blended in 30 the blending tank 32 by introduction in controlled proportions through lines 29 and 30 from the receivers 26 and 28 respectively.

The products of the present invention as described above are also useful as pour point depressants for lowering the pour point of a mineral oil. For example, the addition of a small proportion of a heavy condensation product recovered from the high temperature pyrolysis of a normally gaseous hydrocarbon of the character 40 described above, to a partially dewaxed lubricating oil derived from a paraffin base or a mixed base crude, will materially lower the normal pour point of such lubricating oil. It is recognized that the presence of a certain amount of wax 45 in a paraffin base or mixed base lubricating oil may be beneficial from the standpoint of providing a comparatively flat temperature-viscosity curve. However, the pour point of such a partially dewaxed lubricating oil of this character 50 is normally high, such as around 25° F. or above. Consequently, it is of advantage to add to the oil a material which will have the effect of reducing the pour test or cold test to the desired extent without the necessity of entirely removing 55 the remaining wax. The condensation product produced as outlined above may be added directly to a lubricating stock; or an extract of the condensation product may be first prepared and this extract added to the lubricating stock. 60 Thus, a small proportion of the mineral oil to be treated, or other lubricating oil, may be used to form a concentrate of the active pour point depressant materials in the condensation product; and this concentrate can then be added in pre- 65 determined proportions to a larger body of the oil to be treated. Again, different solvents may be employed to produce an extract of the condensation product. Suitable solvents include benzene, xylene, toluene and various aliphatic monohydric alcohols from methyl to the amyl alcohols. The proportions in which the pour point depressant material is added to the mineral lubricating oil can be varied widely. However, it is 70 usually desirable to add only that proportion 75

which will lower the pour point to the required low temperature. Generally, less than 5% by weight of the pour point depressant material is used; and often as little as a fraction of 1%, such as about  $\frac{1}{2}\%$  or less, is sufficient.

The products of the present invention are also useful in connection with the removal of wax from a wax bearing hydrocarbon oil. Thus, the addition of a small proportion of the heavy condensate, or extracts thereof, recovered from the high temperature pyrolysis of a normally gaseous hydrocarbon of the character set out above, to a wax bearing oil, is found to modify wax crystal formation upon chilling of the oil, to thereby facilitate separation of the wax from the oil by centrifuging or cold settling. It is also found that the addition of a wax crystal modifying material of this character to a wax bearing oil results in substantially increasing filtering rates, where the wax is separated from the chilled oil by filtration. The employment of products of the present invention along with a solvent in which both the solid and normally liquid constituents are soluble at elevated temperatures of the order of  $100^{\circ}$  F. or above, and in which the normally liquid constituents are soluble but the normally solid constituents or waxes are substantially completely insoluble at lowered temperatures of the order of  $0^{\circ}$  F. to  $-20^{\circ}$  F., is found particularly beneficial. Various solvents of this character may be employed, such for example, as acetone, ethylene dichloride, methyl ethyl ketone, liquid sulphur dioxide, naphtha, propyl alcohol and the like. Mixtures of such selective and non-selective solvent liquids are also satisfactory. For example, a very suitable solvent mixture capable of serving as a dewaxing solvent consists of acetone and benzol, for instance in the proportions of 35% acetone and 65% benzol. Another very suitable solvent mixture, particularly for the dewaxing of residual oils, consists of about 28-35% acetone, 47-57% benzol and 15-18% toluol.

By way of example, a proportion of 1 to 10% by weight of the heavy condensation product obtained from the pyrolysis of oil gas, as described above, may be added to a wax bearing lubricating oil fraction, together with a solvent mixture of 35% acetone and 65% of benzol in the proportions of one part of oil to three parts of the acetone-benzol mixture. The oil is then chilled to a temperature of around  $0^{\circ}$  to  $-10^{\circ}$  F. and subjected to settling at this temperature. The wax constituents settle rapidly from the mixture, the supernatant liquid layer of oil and solvent may be drawn off, and the solvent removed therefrom by distillation. According to another method of operation, the chilled mixture may be subjected to centrifuging with satisfactory separation of the wax from the oil. In still another method of operation, the chilled mixture may be subjected to dewaxing by pressure filtration, and the filtering rates be markedly increased over the rates obtained when the condensation product of the present invention is not added. Where a solvent mixture of the character of acetone-benzol or acetone-benzol-toluol is employed, the resulting wax free oil is found to have a pour test of around  $0^{\circ}$  F. when chilled only to about  $0^{\circ}$  F. or slightly below.

Very satisfactory results are also secured by adding to the wax bearing oil a filter aid material, such as an acid treated clay or fuller's earth. This is found beneficial when used in conjunc-

tion with the wax crystal modifying material and also with the solvent or solvent mixture.

Obviously many modifications and variations of the invention, as hereinbefore set forth, may be made without departing from the spirit and scope thereof, and therefore only such limitations should be imposed as are indicated in the appended claims.

I claim:

1. A lubricating oil possessing a green fluorescence, comprising a mixture of a petroleum lubricating oil with a minor proportion of a heavy condensate recovered from the high temperature pyrolysis of a normally gaseous hydrocarbon. 10
2. A lubricating oil possessing a green fluorescence, comprising a mixture of a petroleum lubricating oil with a minor proportion of a heavy condensate recovered from the high temperature pyrolysis of fixed gases from a cracking still. 15
3. A lubricating oil possessing a green fluorescence, comprising a mixture of a petroleum lubricating oil with a minor proportion of a heavy condensate recovered from the high temperature pyrolysis of natural gas. 20
4. A lubricating oil possessing a green fluorescence, comprising a mixture of a petroleum lubricating oil with a minor proportion of a heavy condensate recovered from the high temperature pyrolysis of oil refinery waste gases. 25
5. A lubricating oil possessing a green fluorescence, comprising a mixture of a petroleum lubricating oil normally deficient in bloom, with an amount up to 2% by weight of a heavy condensate formed by pyrolysis at temperatures in excess of  $1150^{\circ}$  F. of a normally gaseous hydrocarbon sufficient to impart the said green fluorescence to the lubricating oil. 30
6. A lubricating oil possessing a green fluorescence, comprising a mixture of a petroleum lubricating oil with a minor proportion of a blend 40 of heavy condensates formed by high temperature pyrolysis of a normally gaseous hydrocarbon, one condensate of the blend being formed by pyrolysis at a different temperature from that of another condensate to thereby give a resulting blend of a controlled color and bloom. 45
7. A lubricating oil possessing a green fluorescence, comprising a mixture of a petroleum distillate lubricating oil which is normally deficient in bloom, with an amount up to 2% by weight of a heavy condensate oil recovered from the pyrolysis of oil gas at temperatures of  $1450^{\circ}$ - $1700^{\circ}$  F., sufficient to impart the said green fluorescence to the lubricating oil. 50
8. A lubricating oil possessing a green fluorescence, comprising a mixture of petroleum distillate lubricating oil, with an amount up to 2% by weight of a blend of heavy condensate oils formed by high temperature pyrolysis of oil gas sufficient to impart the said green fluorescence to the lubricating oil, one condensate oil resulting from pyrolysis at a temperature of  $1450^{\circ}$ - $1500^{\circ}$  F., and another condensate oil resulting from pyrolysis at a temperature of  $1600^{\circ}$ - $1700^{\circ}$  F. 55
9. The method of producing a green bloom lubricating oil, which comprises passing a normally gaseous hydrocarbon through a heating zone maintained at a temperature in excess of  $1150^{\circ}$  F. to pyrolyze the gas, cooling the pyrolyzed gas to recover therefrom a heavy condensate which is concentrated in green bloom imparting material, and adding a proportion of the heavy condensate to a petroleum lubricating oil. 65
10. The method of producing a green bloom lubricating oil, which comprises passing one por- 75

- tion of a normally gaseous hydrocarbon through a heating zone maintained at a temperature in excess of 1150° F. to pyrolyze the gas, passing another portion of a normally gaseous hydrocarbon through a heating zone maintained at a different temperature but also in excess of 1150° F. to pyrolyze the gas, cooling the pyrolyzed gases to recover therefrom heavy condensates which are concentrated in green bloom imparting materials, and adding the condensates in controlled proportions to a petroleum lubricating oil to impart to the latter a controlled color and bloom.
11. The method of producing a green bloom lubricating oil, which comprises passing one portion of oil gas through a heating zone maintained at a temperature of 1450°-1500° F. to pyrolyze the gas, passing another portion of oil gas through a heating zone maintained at a temperature of 1600°-1700° F. to pyrolyze the gas, cooling the pyrolyzed gases to recover therefrom heavy condensates which are concentrated in green bloom imparting materials, and blending controlled proportions of each of the heavy condensates with a petroleum distillate lubricating oil which is normally deficient in the property of bloom to impart to the latter a green bloom of controlled shade.
12. A lubricating oil having a low pour point, comprising a mixture of a partially dewaxed lubricating oil normally having a higher pour point with a small proportion of a heavy condensate recovered from the high temperature pyrolysis of a normally gaseous hydrocarbon.
13. A lubricating oil of improved character comprising a mixture of a petroleum lubricating oil with a minor proportion of a heavy condensate boiling essentially above 400° F. recovered from the high temperature pyrolysis of a normally gaseous hydrocarbon.
14. A lubricating oil possessing a green fluorescence, comprising a mixture of a petroleum lubricating oil with a minor proportion of a heavy condensate recovered from the high temperature pyrolysis of a normally gaseous unsaturated hydrocarbon.

CHARLES C. TOWNE.